

# United States Patent Office

2,853,382  
Patented Sept. 23, 1958

1

2,853,382

## ALLOY COMPOSITIONS

John V. Klochkov, New York, N. Y.

No Drawing. Application July 24, 1957  
Serial No. 673,760

3 Claims. (Cl. 75—175)

These inventions relate to new and improved alloy compositions more particularly to alloy compositions which simulate in appearance a precious metal such as silver.

My new alloy compositions yield silver-like alloys which are valuable metallurgical compounds, and which are fully equivalent for industrial and technological purposes. Especial simulations of the precious metal silver: they can be used to replace the precious metal in dental fields, art articles and silverware industry.

The three alloys according to the invention consist of the following metals by weight:

| Alloy A: | Percent |
|----------|---------|
| Tin      | 42.3    |
| Nickel   | 21.1    |
| Chromium | 18.6    |
| Mercury  | 18.0    |

| Alloy B: | Percent |
|----------|---------|
| Tin      | 59.3    |
| Bismuth  | 13.1    |

| Alloy C: | Percent |
|----------|---------|
| Cobalt   | 15.0    |
| Mercury  | 12.6    |

| Alloy C: | Percent |
|----------|---------|
| Tin      | 27.4    |
| Lead     | 32.0    |
| Cobalt   | 9.1     |
| Chromium | 16.1    |
| Mercury  | 15.4    |

10 I claim:

1. An alloy consisting of the following metals by weight:

| Alloy A: | Percent |
|----------|---------|
| Tin      | 42.3    |
| Nickel   | 21.1    |
| Chromium | 18.6    |
| Mercury  | 18.0    |

2. An alloy consisting of the following metals by weight:

| Alloy B: | Percent |
|----------|---------|
| Tin      | 59.3    |
| Bismuth  | 13.1    |
| Cobalt   | 15.0    |
| Mercury  | 12.6    |

3. An alloy consisting of the following metals by weight:

| Alloy C: | Percent |
|----------|---------|
| Tin      | 27.4    |
| Lead     | 32.0    |
| Cobalt   | 9.1     |
| Chromium | 16.1    |
| Mercury  | 15.4    |

No references cited.